# EUROPEAN PATENT SPECIFICATION

(11) **EP 1 712 580 B1**
(45) Date of publication and mention of the grant of the patent: **10.12.2008**
(21) Application number: 06006673.5
(22) Date of filing: 30.03.2006
(51) Int. Cl.: C08G 65/00, C10M 107/20

(54) **Additives for fluorinated oils**
Zusatz für fluoriertes Öl
Additive d'huiles fluorées

(30) Priority: 14.04.2005 IT MI20050646
(43) Date of publication of application: 18.10.2006
(73) Proprietor: Solvay Solexis S.p.A., 20121 Milano (IT)
(72) Inventor: Russo, Antonio, 20100 Milano (IT); Maccone, Patrizia, 20127 Milano (IT)
(74) Representative: Sama, Daniele

(56) References cited:
- US-A- 5 942 598
- US-A- 6 156 937

## Description

The present invention relates to additives for lubricating oils and greases capable to improve their thermal stability in the presence of metals and in oxidative environment (for example air) and their preparation process.

Particularly the invention relates to additives having a perfluoropolyether structure capable to stabilize lubricants, such as oils and greases, preferably having a perfluoropolyether structure, in combination with to the capability of conferring good anti-rust properties and good stability (high shelf life) to storage at 25°C, i.e. without phase separation.

It is known in the prior art that perfluoropolyethers have a good chemical and thermal stability, and are used as lubricating oils and greases, or as hydraulic fluids in applications where a broad thermal rating is required, and in particular severe conditions, for example in contact with corrosive compounds or with ionizing radiations. However these lubricants show the drawback that in some extremely drastic operating conditions, as for example at temperatures higher than 280°C, in oxidative environment (for example air) and in the presence of metals, tend to decompose showing a limited thermal stability.

The decomposition process in the above described conditions brings to the fragmentation of the perfluoropolyether chains or, in some cases, to the total decomposition of the lubricant itself, thus compromizing the lubricant performances.

Furthermore the fluid decomposition is generally associated with a progressive corrosion of the metal itself.

It is also known in the prior art that the resistance to oxidation of oils and greases having a pefluoropolyether structure, at high temperatures in the presence of metals, can be improved with the use of specific stabilizing additives. They must have as peculiarity a good compatibility with the perfluoropolyether oil. Stabilizing additives containing phosphor and fluorinated substituents are known.

USP 4,681,693 describes stabilizers for perfluoropolyether lubricants having a backbone formed of arylphosphines units, or their derivatives, linked to perfluoropolyether chains through oxygen or sulphur atoms. These compounds are prepared with a multistep process comprising intermediates difficult to be prepared. Therefore this process is hardly industrially usable.

EP 597,369 describes stabilizers for phosphazene derivatives based perfluoropolyether lubricants, having contemporaneously on the phosphazene ring both aromatic groups and (per)fluoropolyether chains. The synthesis of the stabilizers is not selective and does not allow to obtain an additive having a well defined chemical structure. Besides the phosphazene precursor is very expensive and therefore disadvantageous from an industrial point ov view. Tests carried out by Applicant have shown that these compounds have a low stability to storage.

USP 5,326,910 describes perfluoropolyether phosphotriazines as stabilizers for perfluoropolyether oils. These derivatives are obtained by a synthesis requiring many steps and reactants difficult to prepare, as perfluorinated epoxides.

In USP 5,550,277 stabilizers for perfluoropolyether lubricants having the structure of aromatic phosphates or phosphonates substituted by perfluoropolyether chains are described. The synthesis process is very complicated and requires many steps and the use of organometallic reactants, as for example butyl lithium, which, as well known, are difficult to use in industry for plant safety.

In the patent application WO 99/51,612 phosphoric esters, in particular arylphosphates, are described, wherein at least one of the substituents is a perfluoropolyether chain. In the preparation of said additives aromatic chloroesters are used. These compounds have the drawback to be very expensive. Besides, as described in the examples of this document, the phosphoric esters are obtained by reaction of aromatic alcohols with POCl₃, which is toxic and scalding, thus requiring specific equipments for the use on industrial scale.

The stabilizers containing phosphor described so far, although having good stabilizing properties, are however obtained with synthesis processes comprising various steps, some of them require the use of expensive and/or difficult to prepare reactants, requiring operating conditions or technological solutions of difficult management on industrial scale. Besides some of them show a poor stability to storage.

Not containing phosphor stabilizing additives for perfluoropolyether lubricants are also known.

For example in USP 5,942,598 oligomers having a perfluoroalkylenether-triazine structure are described, as lubricants having a good stability to the oxidation in the presence of metals. These oligomers can also be used as stabilizing additives for oils and greases having a perlfuoropolyether structure. However their synthesis requires various steps, some of them require the use of precursors of difficult preparation, with a yield in the final product lower than 40%, and therefore disadvantageous also from an economic point of view. Nothing is said on the anti-rust properties of said compounds.

In patent appliction EP 1,354,932 in the name of the Applicant, stabilizing additives having a perfluoropolyether structure not containing phosphor and having aryl end groups containing NO₂ groups are described. The additives are used to stabilize perfluoropolyether oils and greases in thermooxidative environment in the presence of metals. Tests carried out by the Applicant have shown that, even having good stabilizing performances, these additives show however the inconvenience of phase separation at room temperature. Therefore the compositions containing said additives have poor shelf life.

The need was therefore felt to have available additives:
- capable to stabilize fluorinated lubricants, in particular having a perfluoropolyether structure, at high temperatures in oxidative environment and in the presence of metals;
- showing anti-rust properties;
- stable in fluorinated lubricating oils or greases at room temperatures without phase separation, thus obtaining compositions stable to storage (high shelf life);
- obtainable by a simple industrial process.
   The Applicant has surprisingly and unexpectedly found particular compounds having a perfluoropolyether structure capable to satisfy the above combination of properties.
   An object of the present invention are compounds comprising perfluoropolyether chains and having at least one aryltriazine end group, of formula:
wherein
- R_{f} is a (per)fluoropolyoxyalkylene chain formed of one or more repeating units, statistically placed along the chain, having the following structure: (CFXO), (CF₂CF₂O) , (CF₂CF₂CF₂O) , (CF₂CF₂CF₂CF₂O), (CR₆R₇CF₂CF₂O), (CF(CF₃)CF₂O), (CF₂CF(CF₃)O), wherein X = F, CF₃; R₆ and R₇, equal to or different from each other, are selected from H, Cl, or perfluoroalkyl from 1 to 4 carbon atoms, said R_{f} having a number average molecular weight in the range 500-10,000, preferably 500-5,000;
- W₁, W₂, equal to or different frome ach other, are -F or -CF₃;
- T₁ is equal to -CHAₐ-Bₐ(CH₂CH₂O)ₙₐ- wherein Aₐ = H, CF₃; Bₐ = O, S, NH ; na is an integer from 0 to 6, extremes included;
- T₂ is equal to -F, -CF₃, -C₂F₅, - (C₂F₄)Cl, or a group of formula:
- Q₁, Q₂, equal to or different from each other, are a perfluorooxyalkylene chain of formula:
   -T₁-CFW₁-O-R_{f}-CFW₂-T'₂, wherein T'₂ is equal to -F, -CF₃, -C₂F₅, -(C₂F₄)Cl; T₁, W₁ and W₂ have the above meaning;
or a group of formula: wherein B is equal to 0, S, NH; R₁, R₂, R₃, R₄, R₅, equal to or different from each other, are selected from H, F, NO₂, CN, linear or branched C₁-C₈ perfluoroalkyl, carboxyl, phenyl (Ph), O-Ph, NH-Ph, S-Ph;
with the proviso that at least one of Q₁ and Q₂ is equal to the group:

The preferred perfluoropolyether chain R_{f} is selected from the following structures:
(A) -(CF₂CF(CF₃)O)ₐ(CFXO)_{b}- or
   - (CF₂CF (CF₃) O) ₐ (CFXO) _{b}-CF₂ (R'_{f}) CF₂-O- (CF₂CF (CF₃) O) ₐ(CFXO) _{b}-
   wherein R'_{f} is a fluoroalkylene group from 1 to 4 C atoms; X is F or CF₃; a and b are integers such that the number average molecular weight is within the above range; a/b is between 10 and 100, b being different from 0;
(B) - (CF₂CF₂O)_{c}(CF₂O)_{d}(CF₂ (CF₂) _{z}O) ₕ-
   wherein c, d and h are integers such that the number average molecular weight is within the above range; c/d, d being different from 0, is between 0.1 and 10; h/ (c+d), (c+d) being different from 0, is between 0 and 0.05; z is 2 or 3; h can also be equal to 0;
(C) - (CF₂CF(CF₃)O)ₑ (CF₂CF₂O) _{f} (CFXO)_{g}-
   wherein X is F or CF₃; e, f, g are integers such that the number average molecular weight is in the above range; e/(f+g) is between 0.1 and 10, (f+g) being different from 0; f/g is between 2 and 10;
(D)-(CF₂(CF₂)_{z}O)ₛ-
   wherein s is an integer such as to give the above molecular weight, z has the already defined meaning;
(E) - (CR₆R₇CF₂CF₂O)_{j'} - or
   - (CR₆R₇CF₂CF₂O)_{p'}-R'_{f}-O- (CR₆R₇CF₂CF₂O)_{q'}-
   wherein R₆ and R₇ are equal to or different from each other and selected from H, Cl or perfluoroalkyl from 1 to 4 C atoms; R'_{f} is a fluoroalkylene group from 1 to 4 C atoms; j', p' and q' are integers such as to have a molecular weight as the above mentioned one;
(F) -(CF(CF₃)CF₂O)_{j"}-
   j" being an integer such as to give the above molecular weight.

Preferably the R_{f} structures in the compounds of formula (I) are selected between the structures (A) and (B).

The Applicant has surprisingly and unexpectedly found that the compounds of the invention can be used as additives of perfluorinated lubricants, as perfluoropolyether oils or perfluoropolyether base greases, to confer an improved thermal stability to the lubricant in oxidative environment and in the presence of metals in combination with good anti-rust properties and good shelf life at 25°C.

The pefluoropolyether compounds having at least one aryltriazine end group are transparent and odourless viscous liquids.

A further object of the present invention are lubricating compositions comprising:
- from 99.95 to 90% by weight, preferably from 99.5 to 95%, of a perfluoropolyether oil or a PFPE based grease on perfluoropolyether oils;
- from 0.05 to 10% by weight, preferably from 0.5 to 5% by weight, of at least one of the triazine compounds of formula (I).

Examples of perfluoropolyether oils are those belonging to the following classes:
(1) E-O-[CF₂CF(CF₃)O]_{m'} (CFXO)_{n'}-E'
   wherein
   X is equal to -F or -CF₃;
   E and E', equal to or different from each other, are selected from -CF₃, -C₂F₅ or -C₃F₇;
   m' and n' are integers such that the m'/n' ratio is between 20 and 1,000, n' being different from 0, and the viscosity of the product at 20°C is between 10 and 4.000 cSt; the units being statistically distributed along the backbone.
   These polymers can be obtained by perfluoropropene photooxidation, as described in GB 1,104,432, and by subsequent conversion of the end groups, as described in GB 1,226,566.
(2) C₃F₇O-[CF(CF₃)CF₂O]_{o'}-D
   wherein
   D is equal to -C₂F₅ or -C₃F₇;
   o' is an integer such that the viscosity of the product is within the range indicated under (1).
   These polymers can be prepared by ionic oligomerization of perfluoropropyleneoxide and subsequent treatment with fluorine as described in USP 3,242,218.
(3) {C₃F₇O-[CF(CF₃)CF₂O]_{p'}-CF(CF₃)-}₂
   wherein
   p' is an integer such that the viscosity of the product is within the range indicated under (1).
   These products can be obtained by ionic telomerization of perfluoropropyleneoxide and subsequent photochemical dimerization as reported in USP 3,214,478.
(4) E-O-[CF₂CF(CF₃)O]_{q'} (C₂F₄O)_{r'} (CFX)_{s'}-E'
   wherein
   X is equal to -F or -CF₃;
   E and E', equal to or different from each other, are selected from -CF₃, -C₂F₅ or -C₃F₇;
   q', r' and s' are integers, including 0, so that the viscosity of the product is in the range indicated under (1) .
   These polymers can be obtained by photooxidation of a mixture of C₃F₆ and C₂F₄ and subsequent treatment with fluorine as described in USP 3,665,041.
(5) E-O-(C₂F₄O)_{t'} (CF₂O)_{u'}-E'
   wherein
   E and E', equal to or different from each other, are selected from -CF₃, -C₂F₅ or -C₃F₇;
   t' and u' are integers such that the t'/u' ratio is between 0.1 and 5, u' being different from 0, and the viscosity of the product is in the reported range under (1).
   These polymers are obtained by photooxidation of C₂F₄ as reported in USP 3,715,378 and subsequent treatment with fluorine as described in USP 3,665,041.
(6) E-O- (CF₂CF₂CF₂O)_{v'} -E'
   wherein
   E and E', equal to or different from each other, are selected from -CF₃, -C₂F₅ or -C₃F₇;
   v' is a number such that the viscosity of the product is in the above reported range under (1).
   These polymers are obtained as reported in EP 148,482.
(7) D-O-(CF₂CF₂O)_{z'}-D'
   wherein
   D and D', equal to or different from each other, are selected from -C₂F₅ or -C₃F₇;
   z' is an integer such that the viscosity of the product is within the above reported range under (1).
   These polymers can be obtained as reported in USP 4,523,039.
(8) E₁-O (CF₂O) ₙ (CF₂CF₂O) ₘ- (CF₂CF₂CF₂O) p (CF₂CF₂CF₂CF₂O) _{q}-E₂
   wherein
   E₁ and E₂ are perfluoroalkyl end groups equal to or different from each other, having formula - (CF₂)_{z}CF₃, wherein z is an integer from 0 to 3; n, m, p, q are integers such that the viscosity is as defined under (1) , m/n is between 2 and 20, n being different from 0, preferably between 2 and 10;
   the ratio (p+q)/(m+n+p+q) is between 0.05 and 0.2, (m+n+p+q) being different from 0; n/(m+n+q+p) ranges between 0.05 and 0.4, (m+n+p+q) being different from 0.

These are obtained according to EP 1,454,938.

The preferred perfluoropolyether oils are those of the class (1), (4), (5) and (8).

The above mentioned perfluoropolyethers of the classes from (1) to (8) have perfluoroalkyl end groups, are liquid with a very low vapour pressure value and have a viscosity, at 20°C, generally between 10 and 100,000 cSt, preferably between 40 and 2,000 cSt.

The perfluoropolyethers usable for preparing oils and greases are available on the market as for example FOMBLIN® (Solvay Solexis).

The lubricant compositions of the present invention have a high shelf life at room temperature and do not visually show any substantially phase separation for long periods of time.

The compositions of the present invention can also contain other additives commonly used in perfluoropolyether lubricant formulations, as for example anti-wear additives.

A further object of the present invention is a process to obtain the triazine compounds of formula (I) comprising the following stages:

### STAGE A)

i) reaction of a perfluoropolyoxyalkylene derivative having formula

   T"₁-CFW₁-O-R_{f}-CFW₂-T"₂ (II)

   wherein
   Rf, W₁ and W₂ have the above meaning;
   T"₁ and T"₂ can be equal to or different from each other, having general formula equal to -CHAₐ-Bₐ(CH₂CH₂O)ₙₐ-H, wherein Aₐ = H, CF₃; Bₐ = O, S, NH; na is an integer from 0 to 6, extremes included; or selected from F, CF₃, C₂F₅, (C₂F₄)Cl, with the proviso that at least one of the two end groups T"₁ and T"₂ is equal to -CHAₐ-Bₐ(CH₂CH₂O)ₙₐ-H, preferably is selected from O-CH₂OH, O-CH₂SH, O-CH₂NH₂, CH(OH)CF₃;
   with
   a trihalo-triazine of formula: wherein J = Cl, F, preferably Cl;
   at a temperature between 0° and 10°C, wherein the ratio between the equivalents of the compound (II) and the moles of (III) is equal to 1:1, in the presence of a solvent inert under the reaction conditions, capable to solubilize the reactants, and in the presence of an organic or inorganic base, preferably maintaining the reaction mixture under stirring;
ii) reaction of the product obtained in i) with an equivalent of a derivative of formula:

   Q-H (IV)

   wherein Q has the above reported meaning for Q₁ and Q₂;
   at a temperature in the range 25°-35°C;
iii) reaction of the product obtained in ii) with an equivalent of a compound of formula (IV), equal to or different from the one used in step ii), at a temperature in the range 65°C-100°C, preferably 70°C-90°C;

### STAGE B)

separation of the organic phase of the reaction mixture obtained in A) from the aqueous phase and subsequent separation, preferably by filtration, of the organic phase to remove the residual organic or inorganic insoluble salts;

### STAGE C)

several washings of the liquid organic phase with acid water and subsequent separation of the obtained compound of formula (I) from the organic solvent, for example by evaporation.

In stage A) the inert solvent is preferably selected from toluene, xylene, hexafluoroxylene, acetone, diethyl-ketone, etc. The used solvent amount is depending on the reactant solubility in the solvent itself. In stage A) as inorganic base, NaOH, KOH, Na₂CO₃, K₂CO₃ can be used; as organic base, 2,6-dimethylpyridine, 2-methylquinoline, 2,4,6-trimethylpyridine (collidine) can be used. Preferably as base 2,4,6-trimethylpyridine is used.

The ratio between the equivalents of the base and the sum of the equivalents of compounds (II) and (IV) used in the above mentioned three steps of stage (A) is in the range 1:1-2:1, preferably 1:1-1.5:1.

The reaction times for each step are between 2 and 8 hours, preferably between 4 and 6 hours.

The compounds of formula (II) are known in the prior art, for example from USP 6,509,509 and USP 5,124,058.

The reactants having the structure (III), (IV) are known and commercially available.

The process of the present invention results particularly advantageous as the selective substitution of only one halogen atom of the triazine ring (III) which takes place in each step i), ii), iii) of stage A) allows the highly selective substitution of the halogen atoms of the triazine reactant (III) obtaining additives having a predetermined chemical structure.

Said selective process allows furthermore to obtain the triazine compounds of formula (I) with a yield higher than about 90%.

As said, the additives of the present invention do not contain phosphor, are obtainable with a defined chemical structure in high yields by a simple and highly selective process. Said additives allow furthermore to broaden the application field of the perfluoropolyether lubricants in thermooxidative environment in the presence of metals, in particular at temperatures higher than 280°C, in combination with anti-rust properties and high shelf life at 25°C.

The lubricating compositions comprising the additives of the present invention can be used in the presence of metals and in oxidative environment (in the presence of air and oxygen) at high temperatures, higher than 200°C, without any substantial lubricant degradation phenomenon. In particular the lubricating compositions containing the additives of the present invention can be used even at temperatures of about 300°C.

Besides, as said, the compositions of the present invention have the advantage to be stable to storage at room temperature for long periods of time, thus overcoming the prior art drawbacks.

The Applicant has surprisingly and unexpectedly found that the compounds of the present invention, although containing non fluorinated substituents as the phenol groups, are dispersible in fluorinated oils at room temperature and do not show any substantial phase separation, thus allowing stability to storage (i.e. high shelf life).

As said, the additives of the present invention can be used in lubricating oils and greases. In particular the preferred greases are the fluorinated ones, more preferably perfluoropolyether base greases. In the case of perlfuoropolyether-based lubricating greases, the compositions contain, besides the additive of the present invention and the perfluoropolyether oil belonging to one or more of the above mentioned classes, as an essential component, a thickener, in the amounts used in the prior art, as for example PTFE, sodium terephthalamate, calcium or lithium soaps, polyurea. Besides, said compositions can also contain other additives commonly used in grease technology, as talc, inorganic fillers, anti-wear additives. In the case of PTFE used as a thickener, the polymer primary particle sizes, measured by electronic scanning microscopy (SEM); are between 0.02 and 0.25 micron. Said particles can be obtained, for example, by known microemulsion, emulsion, suspension polymerization processes.

The present invention will be better illustrated by the following Examples, which have a merely illustrative and not limitative purpose of the invention.

### EXAMPLES

### CHARACTERIZATION

### Microoxidation test

The microoxidation test reported in the Examples has been carried out by using the equipment described in the following publication: Carl E. Snyder, Jr. and Ronald E. Dolle, Jr., ASLE Transactions, 13(3), 171-180 (1975)*.* The used operating conditions were the following:
- Test temperature :: 300°C
- Air flow :: 1 l/h
- Metals dipped in the fluid:: stainless steel (AISI 304)
and Ti alloy (Al 6%, V 4%)
- Test duration :: 24, 48, 72 hours

The lubricating composition to be tested is introduced in the glass test tube of the equipment shown in the reference Fig. 1, and the whole is weighed and brought to the test temperature. When 24, 48 or 72 hours have elapsed, depending on the test kind, the glass test tube, cooled at room temperture, is weighed again. The difference of weight before and after the heating determines the per cent weight loss of the composition under examination.

After the test the surface aspect of the metals which have been dipped in the tested composition is visually evaluated.

### Test in fog chamber (anti-rust)

A series of carbon steel (C15) (UNI) sheets having 50x100x2 mm sizes are prepared by polishing with abrasive papers (400-800 mesh) followed by cleaning and degreasing with a cloth soaked in n-hexane, and then dried. These sheets are treated by dip-coating in the"test dispersion and then placed in the fog chamber. The fog chamber is formed of one sprayer, connected to a water reserve, which, by compressed air (P = 3 atm) is capable to saturate with moisture the chamber at the temperature of 35°C. The sheets are left in the chamber closed and saturated with moisture and are controlled at time regular intervals by visual inspection up to the appearance of stains on the surface. The test evaluation is expressed according to the following classification:
(0) no rust stain;
(1) one/three corrosion spots having a diameter lower than 1 mm;
(2) three stains having a diameter higher than 1 mm or more stains having a diameter lower than 1 mm for a total of corroded surface lower than 1%;
(3) four or five stains having a diameter higher than 1 mm or more stains having a diameter lower than 1 mm for a total of corroded surface between 1% and 5%;
(4) corroded surface between 5% and 10%;
(5) corroded surface higher than 10%.

### Kinematic viscosity of the perfluoropolyether oil

The kinematic viscosity has been measured by capillary viscometer Cannon-Fenske according to the ASTM D445 method.

### PREPARATION OF THE ADDITIVES

### EXAMPLE 1

### Preparation of the additive (I) of formula:

wherein c and d are integers such that c/d = 2 and OCH₂CF₂(OCF₂)_{d}(OCF₂CF₂)_{c}OCF₂CH₂O has an average molecular weight of 1,464

300 g of hexafluoroxylene, 12.7 g (0.068 moles) of 2,4,6-trichlorotriazine and 9 g (0.074 moles) of collidine are introduced in a 1 litre glass flask, equipped with mechanical stirring, thermometer and dripper. The reaction mixture is cooled to 0°C and then 50 g (0.034 moles, 0,068 eq) of HOCH₂CF₂(OCF₂)_{d}(OCF₂CF₂)_{c}OCF₂CH₂OH (MW = 1,466) are slowly dripped, under stirring, maintaining the temperature inside the flask between 0°C and 10°C.

When the alcohol dripping is over, the reaction mixture is kept under these conditions for about 2 hours, then it is brought to room temperature and left under these conditions for further 2 hours.

9 g (0.074 moles) of collidine are then added and the temperature brought to 30°C. Under these conditions 42.8 g (0.068 eq) of Cl(C₃F₆O)ₐCF₂OH (MW = 631) are added by dripping under stirring. When the addition is over, the reaction is allowed to continue for about 4 hours under stirring. Additional 9 g (0.074 moles) of collidine and 6.4 g (0.068 eq) of phenol are then added to the reaction mixture. After the addition, the temperature is brought to 80°C and the reaction is allowed to continue for about 6 hours.

After cooling, the precipitated collidine hydrochloride is then removed from the reaction mixture by filtration.

The liquid organic mass is then washed with 150 g of an aqueous HCl solution at 2% by weight. After separation of the organic phase the solvent is distilled and the product stripped at 130°C/1mmHg for about 4 hours. 96.3 g of product with a yield equal to 92% are thus obtained.

The IR and NMR analyses (¹H, ¹³C and ¹⁹F) confirm the structure and thus the high selectivity of the synthesis.

### EXAMPLE 2

### Preparation of the additive (I) of formula:

wherein c and d are integers such that c/d = 2 and OCH₂CF₂(OCF₂)_{d}(OCF₂CF₂)_{c}OCF₂CH₂O has an average molecular weight of 1,464.

The Example 1 was repeated but by using 9.4 g (0.068 eq) of p-nitrophenol instead of phenol.

97.8 g of product with a yield equal to 91% are thus obtained. The IR and NMR analyses (¹H, ¹³C and ¹⁹F) confirm the structure and thus the high selectivity of the synthesis.

### EXAMPLE 3

### Preparation of the additive of formula:

wherein a is an integer such that T₁'-CFW₁-O(C₃F₆O)ₐ-CFW₂-T₂' has a number average molecular weight equal to 3770; W₁ and W₂ are equal to F or CF₃; T1' is equal to -F, -CF₃, -C₂F₅; T₂' is equal to a 60/40 mixture of -CH(CF₃)O- and -CH₂-O-.

300 g of hexafluoroxylene, 6.35 g (0.034 moles) of 2,4,6-trichlorotriazine and 4.5 g (0.036 moles) of collidine are introduced in a 1 litre glass flask, equipped with mechanical stirring, thermometer and dripper. The reaction mixture is cooled to 0°C and then 128 g (0.034 moles) of the compound (II) T₁'-CFW₁-O(C₃F₆O)ₐ-CFW₂-T₂'-H (MW = 3,771), prepared according to the teaching of USP 5,124,058 herein incorporated by reference, are slowly dripped, under stirring, maintaining the temperature inside the flask between 0°C and 10°C.

When the alcohol dripping is over, the reaction mixture is kept under these conditions for about 2 hours, then it is brought to room temperture and left under these conditions for further 2 hours.

9 g (0.074 moles) of collidine and 9.4 g (0.068 eq) of p-nitrophenol are then added. After the addition, the temperature is brought to 80°C and the reaction is allowed to continue for about 6 hours.

After cooling, the precipitated collidine hydrochloride is then removed from the reaction mxiture by filtration.

The liquid organic mass is then washed with 150 g of an aqueous HCl solution at 2% by weight. After separation of the organic phase the solvent is distilled and the product stripped at 130°C/1mmHg for about 4 hours. 133 g of product with a yield equal to 95% are thus obtained. The IR and NMR analyses (¹H, ¹³C and ¹⁹F) confirm the structure and thus the high selectivity of the synthesis.

### EXAMPLE 4

### Preparation of the additive of formula:

wherein a is an integer such that T₁'-CFW₁-O (C₃F₆O)ₐ-CFW₂-T₂' has a number average molecular weight equal to 1295; W₁ and W₂ are equal to F or CF₃; T1' is equal to -F, -CF₃, -C₂F₅; T₂' is equal to a 60/40 mixture of -CH(CF₃)O and -CH₂-O.

300 g of hexafluoroxylene, 7.1 g (0.038 moles) of 2,4,6-trichlorotriazine and 5 g (0.041 moles) of collidine are introduced in a 1 litre glass flask, equipped with mechanical stirring, thermometer and dripper.

The reaction mixture is cooled to 0°C and then 50 g (0.038 moles) of the compound (II) T₁'-CFW₁-O(C₃F₆O)ₐ-CFW₂-T₂'-H (MW = 1,296), prepared according to the teaching of USP 5,124,058 herein incorporated by reference, are slowly dripped under stirring, maintaining the temperature inside the flask between 0°C and 10°C.

When the alcohol dripping is over, the reaction mixture is kept under these conditions for about 2 hours, then it is brought to room temperature and left under these conditions for further 2 hours.

5 g (0.041 moles) of collidine are then added and the temperature is brought to 30°C. Under these conditions, by dripping under stirring, additional 50 g (0.038 eq) of T₁'-CFW₁-O(C₃F₆O)ₐ-CFW₂-T₂'-H are added. When the addition is over, the reaction is allowed to continue for about 4 hours. Additional 5 g (0.041 moles of collidine and 3.6 g (0.088 eq) of phenol are then added to the reaction mixture. After the addition, the temperature is brought to 80°C and the reaction is allowed to continue.for about 6 hours.

After cooling, the precipitated collidine hydrochloride is then removed from the reaction mixture by filtration.

The liquid organic mass is then washed with 150 g of an aqueous HCl solution at 2% by weight. After separation of the organic phase the solvent is distilled and the product stripped at 130°C/1mmHg for about 4 hours. 98.2 g of product with a yield equal to 92% are thus obtained. The IR and NMR analyses (¹H, ¹³C and ¹⁹F) confirm the structure and thus the high selectivity of the synthesis.

### EXAMPLE 5 (comparative)

### Preparation of a triazine additive

not containing aryl substituents, wherein a is an integer such that T₁'-CFW₁-O(C₃F₆O)ₐ-CFW₂-T₂' has a number average molecular weight equal to 3770; W₁ and W₂ are equal to F or CF₃; T₁' is equal to -F, -CF₃, -C₂F₅; T₂' is equal to a 60/40 mixture of -CH(CF₃)O- and -CH₂-O- .

300 g of hexafluoroxylene, 6.35 g (0.034 moles) of 2,4,6-trichlorotriazine and 13.5 g (0.108 moles) of collidine are introduced in a 1 litre glass flask, equipped with mechanical stirring, thermometer and dripper.

The reaction mixture is cooled to 0°C and then 384 g (0.102 moles) of the compound (II) T₁'-CFW₁-O(C₃F₆O)ₐ-CFW₂-T₂'-H (MW = 3,771) are slowly dripped, under stirring, maintaining the temperature inside the flask between 0°C and 10°C.

When the alcohol dripping is over, the reaction mixture temperature is slowly brought to 80°C and the reaction is allowed to continue for about 6 hours.

After cooling, the precipitated collidine hydrochloride is then removed from the reaction mixture by filtration.

The liquid organic mass is then washed with 150 g of an aqueous HCl solution at 2% by"weight. After separation of the organic phase the solvent is distilled and the product stripped at 130°C/1mmHg for about 4 hours. 370 g of product with a yield equal to 93% are thus obtained. The IR and NMR analyses (¹H, ¹³C and ¹⁹F) confirm the structure and thus the high selectivity of the synthesis.

### APPLICATION TESTS

### EXAMPLE 6

50 g of a perfluoropolyether oil of the class (5), having kinematic viscosity at 20°C of 260 cSt, commercially known as Fomblin® Z25, are added with 0.5 g of the additive of the Example 4 and then introduced in the glass test tube for the microoxidation test, in the presence of metals. After 24 hours at 300°C under the indicated operating conditions, a weight loss of 1.1% was determined.

The metals dipped in the fluid during the test (stainless steel and Ti, Al, V alloy) did not show oxidation/attack signs, but resulted comparable with those not exposed to the treatment.

During the test the composition kept limpid and no development of smokes was observed.

Furthermore the composition obtained by adding the perfluoropolyether oil with the additive of the Example 4 has resulted stable at room temperature and it does not visually show any separation after 168 hours.

### EXAMPLE 7

The Example 6 was repeated but increasing the time of the microoxidation test to 48 hours. At the end of the test a loss of 1.46% by weight was measured.

### EXAMPLE 8

The Example 6 was repeated by using 0.5 g of the additive of the Example 1. After 24 hours at 300°C under the indicated operating conditions a weight loss of 0.98% was measured. The metals dipped into the fluid during the test (stainless steel and Ti, Al, V alloy) do not show oxidation/attack signs, but are comparable with those not exposed to the treatment.

The composition obtained by adding the perfluoropolyether oil with the additive of the Example 1 resulted stable at room temperature and it did not visually show any phase separation after 168 hours.

### EXAMPLE 9

The Example 8 was repeated but increasing the time of the microoxidation test to 48 hours. At the end of the test a loss of 1.6% by weight was measured.

### EXAMPLE 10

The Example 8 was repeated but increasing the time of the microoxidation test to 72 hours. At the end of the test a loss of 2.2% by weight was measured.

### EXAMPLE 11

The Example 6 was repeated by using 0.5 g of the additive of the Example 3. After 24 hours at 300°C under the indicated operating conditions a weight loss of 0.47% was measured. The metals dipped into the fluid during the test (stainless steel and Ti, Al, V alloy) do not show oxidation/attack sings, but are comparable with those not exposed to the treatment.

The composition obtained by adding the perfluoropolyether oil with the additive of the Example 3 resulted stable at room temperature and it did not visually show any separation after 168 hours.

### EXAMPLE 12

The Example 6 was repeated by using 0.5 g of the additive of the Example 2. After 24 hours at 300°C under the indicated operating conditions a weight loss of 0.82% was measured. The metals dipped into the fluid during the test (stainless steel and Ti, Al, V alloy) do not show oxidation/attack signs, but are comparable with those not exposed to the treatment.

The composition obtained by adding the perfluoropolyether oil with the additive of the Example 2 resulted stable at room temperture and it did not visually show any separation after 168 hours.

### EXAMPLE 13 (comparative)

The Example 6 was repeated in the absence of stabilizing additives. During the test a development of white smokes was observed. After 24 hours at 300°C under the indicated operating conditions the oil was completely decomposed.

The metals dipped into the oil during the test (stainless steel and Ti, Al, V alloy) show evident oxidation/attack signs and a remarkable darkening of the surface.

### EXAMPLE 14 (comparative)

The Example 6 was repeated but by using as stabilizing agent 0.5 g of a non triazine stabilizing additive of formula wherein the number average molecular weight of the chain is 1966 and c/d = 1.2, prepared according to the Example 1 of EP 1, 354, 932.

After 24 hours at 300°C under the indicated operating conditions a weight loss of 1.06% was measured. The metals dipped into the fluid during the test (stainless steel and Ti, Al, V alloy) did not show oxidation/attack signs, but were comparable with those not exposed to the treatment.

However the composition obtained by adding the perfluoropolyether oil with the additive having aryl end groups of EP 1,354,932 and not containing triazine rings shows evident phase separation at room temperature already within 24 hours.

### EXAMPLE 15 (comparative)

The Example 6 was repeated but by using as stabilizing agent 0.5 g of the compound of the Example 5 (comparative).

After 24 hours at 300°C under the indicated operating conditions, a weight loss of 49% was measured.

By comparing these data with those of stability of the Examples according to the invention, it results that the compounds containing triazine rings not substituted with aryl groups are not sufficient to guarantee a good stabilizing activity for perfluoropolyether oils in oxidative environment in the presence of metals at high temperatures.

### EXAMPLE 16

A lubricating composition is prepared containing 0,5 g of the additive of the Example 2, 9.5 g of a perfluoropolyether lubricant of structure (1), having kinematic viscosity at 20°C of 40 cSt, commercially known as Fomblin® Y04. Said composition is then diluted with 190 g of a fluorinated solvent commercially known as Galden® SV90.

Then a metal sheet, cleaned according to what reported for the fog chamber test, is treated by dipping for 1 minute in said mixture. Said time elapsed, the sheet is taken and allowed to dry in a ventilated stove for 30 minutes at 60°C to remove the solvent. Then the sheet is placed in the fog chamber for the test.

After 118 hours under the test conditions the sheet does not show corrosion signs.

### EXAMPLE 17 (comparative)

The Example 16 was repeated without adding the invention additive and by using a lubricating mixture formed of 10 g of Fomblin® Y04 oil and 190 g of fluorinated solvent Galden® SV90.

After 118 h under the test conditions the sheet shows an extended corrosion between 5% and 10% of the total surface.

### EXAMPLE 18

The Example 16 was repeated without using the perfluoropolyether oil and by using a mixture formed of 0.5 g of the additive of the Example 2 and 199.5 g of fluorinated solvent Galden® SV90.

After 118 ore under the test conditions the sheet does not show corrosion signs.

### EXAMPLE 19 (comparative)

The Example 16 was repeated by using only 200 g of fluorinated solvent Galden® SV90 (control test).

After 118 hours under the test conditions the sheet shows an extended corrosion higher than 10% of the total surface.

**Table 1: Microoxidation test**

| **Ex.** | **Oil** | **Additive** | **Additive Conc.** (%w/w oil) | **Dispersion Aspect**(at room T) | **Duration test** | **Loss** (%w/w) |
|---|---|---|---|---|---|---|
| 6 | Fomblin Z 25 | Ex. 4 | 1% | Homogeneous after 168h | 24 h | 1.1 |
| 7 | " | " | " | " | 48 h | 1.46 |
| 8 | " | Ex. 1 | " | " | 24 h | 0.98 |
| 9 | " | " | " | " | 48 h | 1.6 |
| 10 | " | " | " | " | 72 h | 2.2 |
| 11 | " | Ex. 3 | " | " | 24 h | 0.47 |
| 12 | " | Ex. 2 | " | " | 24 h | 0.82 |
| 13 comp | " | --- | --- | ---- | 24 h | Decomposed |
| 14 comp | " | EP 1354932 | 1% | Phase Separation after 24h | 24 h | 1.06 |
| 15 comp | " | Triaz. without aryls | | | 24 h | 49 |

**Table 2: Resistance test to corrosion (fog chamber)**

| **Ex.** | **Oil** | **Solvent** | **Additive** | **Concentration** (%w/w of oil) | **Corrosion** |
|---|---|---|---|---|---|
| 16 | Fomblin Y04 | Galden SV 90 | Ex. 2 | 5 | NO |
| 17 comp | Fomblin Y04 | Galden SV 90 | - | - | 5-10% |
| 18 | - | Galden SV 90 | Ex. 2 | - | NO |
| 19 comp | - | Galden SV 90 | - | - | > 10% |

## Claims

1. Compounds comprising perfluoropolyether chains and having at least one aryltriazine end group, of formula: wherein
- R_{f} is a (per)fluoropolyoxyalkylene chain formed of one or more repeating units, statistically placed along the chain, having the following structure: (CFXO), (CF₂CF₂O), (CF₂CF₂CF₂O), (CF₂CF₂CF₂CF₂O), (CR₆R₇CF₂CF₂O), (CF(CF₃)CF₂O), (CF₂CF(CF₃)O), wherein X = F, CF₃; R₆ and R₇, equal to or different from each other, are selected from H, Cl, or perfluoroalkyl from 1 to 4 carbon atoms, said R_{f} having a number average molecular weight in the range 500-10,000, preferably 500-5,000;
- W₁, W₂, equal to or different from each other, are -F or -CF₃;
- T₁ is equal to -CHAₐ-Bₐ(CH₂CH₂O)ₙₐ- wherein Aₐ = H, CF₃;
Bₐ = O, S, NH; na is an integer from 0 to 6, extremes included;
- T₂ is equal to -F, -CF₃, -C₂F₅, -(C₂F₄)Cl, or a group of formula:
- Q₁, Q₂, equal to or different from each other, are a perfluoropolyoxyalkylene chain of formula:
-T₁-CFW₁-O-R_{f}-CFW₂-T'₂,
wherein T'₂ is equal to -F, -CF₃, -C₂F₅,
- (C₂F₄)Cl; T₁, W₁ and W₂ have the above meaning; or a group of formula: wherein B is equal to O, S, NH; R₁, R₂, R₃, R₄, R₅, equal to or different from each other, are selected from H, F, NO₂, CN, linear or branched C₁-C₈ perfluoroalkyl, carboxyl, phenyl (Ph), O-Ph, NH-Ph, S-Ph;
with the proviso that at least one of Q₁ and Q₂ is equal to:

2. Compounds according to claim 1, wherein the perfluoropolyether chain R_{f} is selected from the following structures:
(A) -(CF₂CF(CF₃)O)ₐ(CFXO)_{b}- or
-(CF₂CF(CF₃)O)ₐ(CFXO)_{b}-CF₂(R'_{f})CF₂-O-(CF₂CF(CF₃)O)ₐ(CFXO)_{b}-wherein R'_{f} is a fluoroalkylene group from 1 to 4 C atoms; X is F or CF₃; a and b are integers such that the number average molecular weight is within the above range; a/b is between 10 and 100, b being different from 0;
(B) -(CF₂CF₂O)_{c}(CF₂O)_{d}(CF₂(CF₂)₂O)ₕ-
wherein c, d and h are integers such that the number average molecular weight is within the above range; c/d, d being different from 0, is between 0.1 and 10; h/(c+d), (c+d) being different from 0, is between 0 and 0.05; z is 2 or 3; h can also be equal to 0;
(C) -(CF₂CF(CF₃)O)ₑ(CF₂CF₂O)_{f}(CFXO)_{g}-
wherein X is F or CF₃; e, f, g are integers such that the number average molecular weight is in the above range; e/(f+g) is between 0.1 and 10, (f+g) being different from 0; f/g is between 2 and 10;
(D) -(CF₂(CF₂)₂O)ₛ-
wherein s is an integer such as to give the above molecular weight, z has the already defined meaning;
(E) -(CR₆R₇CF₂CF₂O)_{j'}- or
-(CR₆R₇CF₂CF₂O)_{p'}-R'_{f}-O-(CR₆R₇CF₂CF₂O)_{q'}-
wherein R₆ and R₇ are equal to or different from each other and selected from H, C1 or perfluoroalkyl from 1 to 4 C atoms; R'_{f} is a fluoroalkylene group from 1 to 4 C atoms; j', p' and q' are integers such as to have a molecular weight as the above mentioned one;
(F) -(CF(CF₃)CF₂O)_{j"}-
j" being an integer such as to give the above molecular weight.

3. Compounds according to claim 2, wherein the structures R_{f} are (A) or (B).

4. Use of the compounds of claims 1-3 as thermal stabilizers for fluorinated oils and greases in thermooxidative conditions in the presence of metals.

5. Use of the compounds of claims 1-3 as anti-rust additives for fluorinated oils and greases.

6. Use according to claim 4 as anti-rust additives.

7. Lubricating compositions comprising:
- from 99.95 to 90% by weight, preferably from 99.5 to 95%, of a perfluoropolyether oil or a PFPE based grease on perfluoropolyether oils;
- from 0.05 to 10% by weight, preferably from 0.5 to 5% by weight, of at least one of the triazine compounds of formula (I) of claims 1-3.

8. Compositions according to claim 7, wherein the perfluoropolyether oil is selected from the following classes:
(1) E-O-[CF₂CF(CF₃)O]_{m'}-(CFXO)_{n'}-E'
wherein
X is equal to -F or -CF₃;
E and E', equal to or different from each other, are selected from -CF₃, -C₂F₅ or -C₃F₇;
m' and n' are integers such that the m'/n' ratio is between 20 and 1,000 , n' being different from 0, and the viscosity of the product at 20°C is between 10 and 4.000 cSt; the units being statistically distributed along the backbone.
(2) C₃F₇O-[CF(CF₃)CF₂O]_{o'}-D
wherein
D is equal to -C₂F₅ or -C₃F₇;
o' is an integer such that the viscosity of the product is within the range indicated under (1).
(3) {C₃F₇O-[CF(CF₃)CF₂O]_{p'}-CF(CF₃)-}₂
wherein
p' is an integer such that the viscosity of the product is within the range indicated under (1).
(4) E-O-[CF₂CF(CF₃)O]_{q'}(C₂F₄O)_{r'}(CFX)_{s'}-E'
wherein
X is equal to -F or -CF₃;
E and E', equal to or different from each other, are selected from -CF₃, -C₂F₅ or -C₃F₇;
q', r' and s' are integers, including 0, so that the viscosity of the product is in the range indicated under (1).
(5) E-O- (C₂F₄O)_{t'}(CF₂O)_{u'}-E'
wherein
E and E', equal to or different from each other, are selected from -CF₃, -C₂F₅ or -C₃F₇;
t' and u' are integers such that the t'/u' ratio is between 0.1 and 5, u' being different from 0, and the viscosity of the product is in the above reported range under (1).
(6) E-O-(CF₂CF₂CF₂O)_{v'}-E'
wherein
E and E', equal to or different from each other, are selected from -CF₃, -C₂F₅ or -C₃F₇;
v' is a number such that the viscosity of the product is in the above reported range under (1).
(7) D-O-(CF₂CF₂O)_{z'}-D'
wherein
D and D', equal to or different from each other, are selected between -C₂F₅ or -C₃F₇;
z' is an integer such that the viscosity of the product is within the above reported range under (1).
(8) E₁-O(CF₂O)ₙ(CF₂CF₂O)ₘ-(CF₂CF₂CF₂O)ₚ(CF₂CF₂CF₂CF₂O)_{q}-E₂
wherein
E₁ and E₂ are perfluoroalkyl end groups equal to or different from each other, having formula -(CF₂)₂CF₃, wherein z is an integer from 0 to 3; n, m, p, q are integers such that the viscosity is as defined under (1), m/n is between 2 and 20, n being different from 0, preferably between 2 and 10; the ratio (p+q)/(m+n+p+q) is between 0.05 and 0.2, (m+n+p+q) being different from 0; n/(m+n+q+p) ranges between 0.05 and 0.4, (m+n+p+q) being different from 0.

9. Compositions according to claim 8, wherein the perfluoropolyether oils are those of the classes (1), (4), (5) and (8).

10. Compositions according to claims 7-9 comprising the additives commonly used in perfluoropolyether lubricant formulations, preferably anti-wear additives.

11. A process for preparing triazine compounds of formula (I) of claims 1-3 comprising the following stages:
STAGE A)
i) reaction of a perfluoropolyoxyalkylene derivative having formula
T"₁-CFW₁-O-R_{f}-CFW₂-T"₂ (II)
wherein
Rf, W₁ and W₂ have the above meaning;
T"₁ and T"₂ can be equal to or different from each other, having general formula equal to -CHAₐ-Bₐ(CH₂CH₂O)ₙₐ-H, wherein Aₐ = H, CF₃; Bₐ = O, S, NH; na is an integer from 0 to 6, extremes included; or selected from F, CF₃, C₂F₅, (C₂F₄)Cl, with the proviso that at least one of the two end groups T"₁ and T"₂ is equal to -CHAₐ-Bₐ(CH₂CH₂O)ₙₐ-H, preferably is selected from O-CH₂OH, O-CH₂SH, O-CH₂NH₂, CH(OH)CF₃;
with
a trihalo-triazine of formula: wherein J = Cl, F, preferably Cl;
at a temperature between 0° and 10°C, wherein the ratio between the equivalents of the compound (II) and the moles of (III) is equal to 1:1, in the presence of a solvent inert under the reaction conditions, capable to solubilize the reactants, and in the presence of an organic or inorganic base, preferably maintaining the reaction mixture under stirring;
ii) reaction of the product obtained in i) with an equivalent of a derivative of formula:
Q-H (IV)
wherein Q has the above reported meaning for Q₁ and Q₂;
at a temperature in the range 25°-35°C;
iii) reaction of the product obtained in ii) with an equivalent of a compound of formula (IV), equal to or different from the one used in step ii), at a temperature in the range 65°C-100°C, preferably 70°C-90°C;
STAGE B)
separation of the organic phase of the reaction mixture obtained in A) from the aqueous phase and subsequent separation, preferably by filtration, of the organic phase to remove the residual organic or inorganic insoluble salts;
STAGE C)
several washings of the liquid organic phase with acid water and subsequent separation of the obtained compound of formula (I) from the organic solvent, for example by evaporation.

12. A process according to claim 11, wherein in stage A) the inert solvent is selected from toluene, xylene, hexafluoroxylene, acetone, diethyl-ketone.

13. A process according to claims 11-12, wherein in stage A) the inorganic base is selected from NaOH, KOH, Na₂CO₃, K₂CO₃; the organic base is selected from 2,6-dimethylpyridine, 2-methylquinoline, 2,4,6-trimethylpyridine (collidine).

14. A process according to claims 11-13, wherein the base is 2,4,6-trimethylpyridine.

15. A process according to claims 11-14, wherein the ratio between the equivalents of base and the sum of the equivalents of compounds (II) and (IV) used in the three steps of stage (A) is in the range 1:1-2:1, preferably 1:1-1.5:1.

16. Lubricating greases having a perfluoropolyether base comprising the additive of claims 1-3, a perfluoropolyether oil and a thickener, preferably selected from PTFE, sodium terephthalamate, calcium or lithium soaps, polyurea, more preferably PTFE.

17. Greases according to claim 16 comprising talc, inorganic fillers, anti-wear additives.

## Patentansprüche

1. Verbindungen mit Perfluorpolyetherketten und mindestens einer Aryltriazin-Endgruppe der Formel: worin
- R_{f} für eine (Per)fluorpolyoxyalkylenkette aus einer oder mehreren statistisch entlang der Kette angeordneten Wiederholungseinheiten mit der folgenden Struktur steht: (CFXO), (CF₂CF₂O), (CF₂CF₂CF₂O), (CF₂CF₂CF₂CF₂O), (CR₆R₇CF₂CF₂O), (CF(CF₃)CF₂O), (CF₂CF(CF₃)O), worin X = F, CF₃ ; R₆ und R₇ gleich oder voneinander verschieden sind und unter H, Cl oder Perfluoralkyl mit 1 bis 4 Kohlenstoffatomen ausgewählt sind, wobei R_{f} ein zahlenmittleres Molekulargewicht im Bereich von 500-10.000, vorzugsweise 500-5.000, aufweist;
- W₁ und W₂ gleich oder voneinander verschieden sind und für -F oder -CF₃ stehen ;
- T₁ gleich -CHAₐ-Bₐ(CH₂CH₂O)ₙₐ-, worin Aₐ = H, CF₃, ist;
Bₐ = O, S, NH ; na für eine ganze Zahl von 0 bis 6 einschließlich der Extrema steht ;
- T₂ gleich -F, -CF₃, -C₂F₅, -(C₂F₄)Cl oder einer Gruppe der Formel: ist ;
- Q₁ und Q₂ gleich oder voneinander verschieden sind und für eine Perfluorpolyoxyalkylenkette der Formel:
-T₁-CFW₁-O-R_{f}-CFW₂-T'₂
worin T'₂ gleich -F, -CF₃, -C₂F₅, -(C₂F₄)Cl ist und T₁, W₁ und W₂ die oben angegebene Bedeutung besitzen;
oder eine Gruppe der Formel : worin B gleich O, S, NH ist; R₁, R₂, R₃, R₄ und R₅ gleich oder voneinander verschieden sind und unter H, F, NO₂, CN, linearem oder verzweigtem C₁₋C₈₋Perfluoralkyl, Carboxyl, Phenyl (Ph), O-Ph, NH-Ph und S-Ph ausgewählt sind,
stehen ;
mit der Maßgabe, daß mindestens eine der Gruppen Q₁ und Q₂ gleich : ist.

2. Verbindungen nach Anspruch 1, worin die Perfluorpolyetherkette R_{f} unter den folgenden Strukturen ausgewählt ist :
(A) -(CF₂CF(CF₃)O)ₐ(CFXO)_{b}- oder -(CF₂CF(CF₃)O)ₐ(CFXO)_{b}-CF₂(R'_{f})CF₂-O-(CF₂CF(CF₃)O)ₐ(CFXO)_{b}-,
worin R'_{f} für eine Fluoralkylengruppe mit 1 bis 4 C-Atomen steht; X für F oder CF₃ steht; a und b für solche ganze Zahlen stehen, daß das zahlenmittlere Molekulargewicht im obigen Bereich liegt und a/b zwischen 10 und 100 liegt, wobei b von 0 verschieden ist ;
(B) -(CF₂CF₂O)_{c}(CF₂O)_{d}(CF₂(CF₂)_{z}O)ₕ-,
worin c, d und h für solche ganze Zahlen stehen, daß das zahlenmittlere Molekulargewicht im obigen Bereich liegt; c/d zwischen 0,1 und 10 liegt, wobei d von 0 verschieden ist ; h/(c+d) zwischen 0 und 0,05 liegt,
wobei (c+d) von 0 verschieden ist; z für 2 oder 3 steht und h auch gleich 0 sein kann ;
(C) -(CF₂CF(CF₃)O)ₑ(CF₂CF₂O)_{f}(CFXO)_{g}-,
worin X für F oder CF₃ steht ; e, f und g für solche ganze Zahlen stehen, daß das zahlenmittlere Molekulargewicht im obigen Bereich liegt ; e/(f+g) zwischen 0,1 und 10 liegt, wobei (f+g) von 0 verschieden ist; und f/g zwischen 2 und 10 liegt ;
(D) -(CF₂(CF₂)_{z}O)ₛ-,
worin s für eine solche ganze Zahl steht, daß das zahlenmittlere Molekulargewicht im obigen Bereich liegt und z die bereits angegebene Bedeutung besitzt ;
(E) -(CR₆R₇CF₂CF₂O)_{j'}- oder -(CR₆R₇CF₂CF₂O)_{p'}-R'_{f}-O-(CR₆R₇CF₂CF₂O)_{q'}-,
worin R₆ und R₇ gleich oder voneinander verschieden sind und unter H, Cl oder Perfluoralkyl mit 1 bis 4 C-Atomen ausgewählt sind ; R'_{f} für eine Fluoralkylengruppe mit 1 bis 4 C-Atomen steht und j', p' und q' für solche ganze Zahlen stehen, daß ein Molekulargewicht wie das oben erwähnte vorliegt ;
(F) -(CF(CF₃)CF₂O)_{j"},
wobei j" für eine solche ganze Zahl steht, daß sich das obige Molekulargewicht ergibt.

3. Verbindungen nach Anspruch 2, worin die Strukturen R_{f}(A) oder (B) sind.

4. Verwendung der Verbindungen gemäß den Ansprüchen 1-3 als Wärmestabilisatoren für fluorierte Öle und Fette unter thermooxidativen Bedingungen in Gegenwart von Metallen.

5. Verwendung der Verbindungen gemäß den Ansprüchen 1-3 als Rostschutzadditive für fluorierte Öle und Fette.

6. Verwendung nach Anspruch 4 als Rostschutzadditive.

7. Schmiermittelzusammensetzungen, enthaltend :
- 99,95 bis 90 Gew.-%, vorzugsweise 99,5 bis 95%, eines Perfluorpolyetheröls oder eines Fetts auf PFPE-Basis auf Perfluorpolyetherölen ;
- 0,05 bis 10 Gew.-%, vorzugsweise 0,5 bis 5 Gew.-%, mindestens einer der Triazinverbindungen der Formel (I) gemäß den Ansprüchen 1-3.

8. Zusammensetzungen nach Anspruch 7, worin das Perfluorpolyetheröl aus den folgenden Klassen ausgewählt ist :
(1) E-O-[CF₂CF(CF₃)O]_{m'}(CFXO)_{n'}-E',
worin
X gleich -F oder -CF₃ ist ;
E und E' gleich oder voneinander verschieden sind und unter -CF₃, -C₂F₅ und -C₃F₇ ausgewählt sind ;
m' und n' für solche ganze Zahlen stehen, daß das Verhältnis m'/n' zwischen 20 und 1.000 liegt, wobei n' von 0 verschieden ist, und die Viskosität des Produkts bei 20°C zwischen 10 und 4.000 cSt liegt ; wobei die Einheiten statistisch entlang der Hauptkette verteilt sind ;
(2) C₃F₇O-[CF(CF₃)CF₂O]_{o'}-D,
worin
D gleich -C₂F₅ oder -C₃F₇ ist ;
o' für eine solche ganze Zahl steht, daß die Viskosität des Produkts im unter (1) angegebenen Bereich liegt ;
(3) {C₃F₇O-[CF(CF₃)CF₂O]_{p'}-CF(CF₃)-}₂,
worin
p' für eine solche ganze Zahl steht, daß die Viskosität des Produkts im unter (1) angegebenen Bereich liegt ;
(4) E-O-[CF₂CF(CF₃)O]_{q'}(C₂F₄O)_{r'}(CFX)_{s'}-E',
worin
X gleich -F oder -CF₃ ist ;
E und E' gleich oder voneinander verschieden sind und unter -CF₃, -C₂F₅ oder -C₃F₇ ausgewählt sind ;
q', r' und s' für solche ganze Zahlen einschließlich 0 stehen, daß die Viskosität des Produkts im unter (1) angegebenen Bereich liegt ;
(5) E-O-(C₂F₄O)_{t'}(CF₂O)_{u'}-E',
worin
E und E' gleich oder voneinander verschieden sind und unter -CF₃, -C₂F₅ oder -C₃F₇ ausgewählt sind;
t' und u' für solche ganze Zahlen stehen, daß das Verhältnis t'/u' zwischen 0,1 und 5 liegt, wobei u' von 0 verschieden ist, und die Viskosität des Produkts im unter (1) angegebenen Bereich liegt;
(6) E-O-(CF₂CF₂CF₂O)_{v'}-E',
worin
E und E' gleich oder voneinander verschieden sind und unter -CF₃, -C₂F₅ oder -C₃F₇ ausgewählt sind;
v' für eine solche Zahl steht, daß die Viskosität des Produkts im unter (1) angegebenen Bereich liegt ;
(7) D-O-(CF₂CF₂O)_{z'}-D'
worin
D und D' gleich oder voneinander verschieden sind und unter -C₂F₅ oder -C₃F₇ ausgewählt sind;
z' für eine solche ganze Zahl steht, daß die Viskosität des Produkts im unter (1) angegebenen Bereich liegt ;
(8) E₁-O(CF₂O)ₙ(CF₂CF₂O)ₘ-(CF₂CF₂CF₂O)ₚ(CF₂CF₂CF₂CF₂O)_{q}-E₂,
worin
E₁ und E₂ für gleiche oder voneinander verschiedene Perfluoralkylendgruppen der Formel -(CF₂)_{z}CF₃, worin z für eine ganze Zahl von 0 bis 3 steht, stehen ; n, m, p und q für solche ganze Zahlen stehen, daß die Viskosität den unter (1) definierten Wert aufweist, m/n zwischen 2 und 20 liegt, wobei n von 0 verschieden ist, vorzugsweise zwischen 2 und 10 ; das Verhältnis (p+q)/(m+n+p+q) zwischen 0,05 und 0,2 liegt, wobei (m+n+p+q) von 0 verschieden ist; und n/(m+n+p+q) im Bereich zwischen 0,05 und 0,4 liegt, wobei (m+n+p+q) von 0 verschieden ist.

9. Zusammensetzungen nach Anspruch 8, worin es sich bei den Perfluorpolyetherölen um diejenigen aus den Klassen (1), (4), (5) und (8) handelt.

10. Zusammensetzungen nach den Ansprüchen 7-9, die die in Perfluorpolyether-Schmiermittelformulierungen weithin verwendeten Additive, vorzugsweise Verschleißschutzadditive, enthalten.

11. Verfahren zur Herstellung von Triazinverbindungen der Formel (I) gemäß den Ansprüchen 1-3, umfassend die folgenden Schritte :
STUFE A)
i) Umsetzung eines Perfluorpolyoxyalkylenderivats der Formel
T"₁-CFW₁-O-R_{f}-CFW₂-T"₂ (II)
worin Rf, W₁ und W₂ die oben angegebene Bedeutung besitzen ;
T"₁ und T"₂ gleich oder voneinander verschieden sein können und die allgemeine Formel -CHAₐ-Bₐ(CH₂CH₂O)ₙₐ-H, worin Aₐ = H, CF₃ ; Bₐ = O, S, NH ; na für eine ganze Zahl von 0 bis 6 einschließlich der Extrema steht ; aufweisen oder unter F, CF₃, C₂F₅ oder (C₂F₄)Cl ausgewählt sind, mit der Maßgabe, daß mindestens eine der beiden Endgruppen T"₁ und T"₂ gleich -CHAₐ-Bₐ(CH₂CH₂O)ₙₐ-H ist und vorzugsweise unter O-CH₂OH, O-CH₂SH, O-CH₂NH₂ und CH(OH)CF₃ ausgewählt ist;
mit einem Trihalogentriazin der Formel : worin J = Cl, F, vorzugsweise Cl ;
bei einer Temperatur zwischen 0°C und 10°C, wobei das Verhältnis zwischen den Äquivalenten der Verbindung (II) und den Molen von (III) gleich 1:1 ist, in Gegenwart eines unter den Reaktionsbedingungen inerten Lösungsmittels, das zur Solubilisierung der Reaktanten befähigt ist, und in Gegenwart einer organischen oder anorganischen Base, wobei die Reaktionsmischung vorzugsweise unter Rühren gehalten wird ;
ii) Umsetzung des in i) erhaltenen Produkts mit einem Äquivalent eines Derivats der Formel :
Q-H (IV)
worin Q die oben für Q₁ und Q₂ angegebene Bedeutung besitzt ;
bei einer Temperatur im Bereich von 25-35°C ;
iii) Umsetzung des in ii) erhaltenen Produkts mit einem Äquivalent einer Verbindung der Formel (IV), die mit der in Schritt ii) verwendeten Verbindung identisch oder davon verschieden sein kann, bei einer Temperatur im Bereich von 65°C-100°C, vorzugsweise 70°C-90°C ;
STUFE B)
Trennung der organischen Phase der in A) erhaltenen Reaktionsmischung von der wäßrigen Phase und nachfolgende Trennung, vorzugsweise durch Filtration, der organischen Phase zur Entfernung der verbliebenen organischen oder anorganischen unlöslichen Salze ;
STUFE C)
mehrere Wäschen der flüssigen organischen Phase mit saurem Wasser und nachfolgende Abtrennung der erhaltenen Verbindung der Formel (I) von dem organischen Lösungsmittel, beispielsweise durch Eindampfen.

12. Verfahren nach Anspruch 11, bei dem in Stufe A) das inerte Lösungsmittel unter Toluol, Xylol, Hexafluorxylol, Aceton und Diethylketon ausgewählt wird.

13. Verfahren nach den Ansprüchen 11-12, bei dem in Stufe A) die anorganische Base unter NaOH, KOH, Na₂CO₃ und K₂CO₃ ausgewählt wird und die organische Base unter 2,6-Dimethylpyridin, 2-Methylchinolin und 2,4,6-Trimethylpyridin (Collidin) ausgewählt wird.

14. Verfahren nach den Ansprüchen 11-13, bei dem es sich bei der Base um 2,4,6-Trimethylpyridin handelt.

15. Verfahren nach den Ansprüchen 11-14, bei dem das Verhältnis zwischen den Äquivalenten der Base und der Summe der Äquivalente der Verbindungen (II) und (IV), die in den drei Schritten von Stufe (A) verwendet werden, im Bereich von 1:1-2:1, vorzugsweise 1:1-1,5:1, liegt.

16. Schmierfette mit einer Perfluorpolyetherbasis, die das Additiv gemäß den Ansprüchen 1-3, ein Perfluorpolyetheröl und einen Verdicker, vorzugsweise ausgewählt unter PTFE, Natriumterephthalamat, Calcium- oder Lithiumseifen und Polyharnstoff, besonders bevorzugt PTFE, enthalten.

17. Fette nach Anspruch 16, die Talk, anorganische Füllstoffe, Verschleißschutzadditive enthalten.

## Revendications

1. Composés comprenant des chaînes perfluoropolyéther et renfermant au moins un groupe terminal aryltriazine, de formule : dans laquelle
- R_{f} est une chaîne (per)fluoropolyoxyalkylène formée d'un ou de plusieurs motifs récurrents, placés statistiquement le long de la chaîne, présentant la structure suivante : (CFXO), (CF₂CF₂O) (CF₂CF₂CF₂O), (CF₂CF₂CF₂CF₂O), (CR₆R₇CF₂CF₂O), (CF(CF₃)CF₂O), (CF₂CF(CF₃)O), dans laquelle X est un atome de fluor, un groupe CF₃ ; R₆ et R₇, identiques ou différents l'un de l'autre, sont choisis parmi un atome d'hydrogène, un atome de chlore ou un groupe perfluoroalkyle renfermant de 1 à 4 atomes de carbone, ledit R_{f} présentant un poids moléculaire moyen en nombre dans la plage de 500 à 10 000, de préférence de 500 à 5000 ;
- W₁, W₂, identiques ou différents l'un de l'autre, sont un groupe -F ou un groupe -CF₃ ;
- T₁ est un groupe -CHAₐ-Bₐ(CH₂CH₂O)ₙₐ- dans lequel Aₐ est un atome d'hydrogène, un groupe CF₃.
Bₐ est un atome d'oxygène, un atome de soufre, un groupe NH ; na est un entier de 0 à 6, les extrêmes étant inclus ;
- T₂ est un groupe -F, un groupe -CF₃, un groupe -C₂F₅, un groupe -(C₂F₄)Cl, ou un groupe de formule :
- Q₁, Q₂, identiques ou différents l'un de l'autre, sont une chaîne perfluoropolyoxyalkylène de formule :
-T₁-CFW₁-O-R_{f}-CFW₂-T'₂,
dans laquelle T'₂ est un groupe F, un groupe -CF₃, un groupe -C₂F₅, un groupe -(C₂F₄)Cl ; T₁, W₁ et W₂ présentent la signification ci-dessus ;
ou un groupe de formule : dans laquelle B est un atome d'oxygène, un atome de soufre, un groupe NH ; R₁, R₂, R₃, R₄, R₅, identiques ou différents les uns des autres, sont choisis parmi un atome d'hydrogène, un atome de fluor, un groupe NO₂,
un groupe CN, un groupe perfluoroalkyle en C₁-C₈ linéaire ou ramifié, un groupe carboxyle, un groupe phényle (Ph), un groupe O-Ph, un groupe NH-Ph, un groupe S-Ph ;
à condition qu'au moins l'un parmi Q₁ et Q₂ soit un groupe :

2. Composés selon la revendication 1, dans lesquels la chaîne perfluoropolyéther R_{f} est choisie parmi les structures suivantes :
(A) -(CF₂CF(CF₃)O)ₐ(CFXO)_{b}- ou -(CF₂CF(CF₃)O)ₐ(CFXO)_{b}-CF₂(R'_{f})CF₂-O-(CF₂CF(CF₃)O)ₐ (CFXO)_{b}-
dans lesquelles R'_{f} est un groupe fluoroalkylène renfermant de 1 à 4 atomes de carbone ; X est un atome de fluor ou un groupe CF₃ ; a et b sont des entiers tels que le poids moléculaire moyen en nombre soit dans la plage ci-dessus ; a/b est compris entre 10 et 100, b étant différent de 0 ;
(B) -(CF₂CF₂O)_{c}(CF₂O)_{d}(CF₂(CF₂)₂O)ₕ-
dans laquelle c, d et h sont des entiers tels que le poids moléculaire moyen en nombre soit dans la plage ci-dessus ; c/d, d étant différent de 0, est compris entre 0,1 et 10 ; h/(c+d), (c+d) étant différent de 0, est compris entre 0 et 0,05 ; z vaut 2 ou 3 ; h peut également valoir 0 ;
(C) -(CF₂CF(CF₃)O)ₑ(CF₂CF₂O)_{f}(CFXO)_{g}-
dans laquelle X est un atome de fluor ou un groupe CF₃ ; e, f, g sont des entiers tels que le poids moléculaire moyen en nombre soit dans la plage ci-dessus ; e/(f+g) est compris entre 0,1 et 10, (f+g) étant différent de 0 ; f/g est compris entre 2 et 10 ;
(D) -(CF₂(CF₂)_{z}O)ₛ-
dans laquelle s est un entier tel qu'il donne lieu au poids moléculaire ci-dessus, z présente la signification déjà définie ;
(E) -(CR₆R₇CF₂CF₂O)_{j'}- ou
-(CR₆R₇CF₂CF₂O)_{p'}-R'_{f}-O-(CR₆R₇CF₂CF₂O)_{q'}-
dans lesquelles R₆ et R₇ sont identiques ou différents l'un de l'autre et sont choisis parmi un atome d'hydrogène, un atome de chlore ou un groupe perfluoroalkyle renfermant de 1 à 4 atomes de carbone ; R'_{f} est un groupe fluoroalkylène renfermant de 1 à 4 atomes de carbone ; j', p' et q' sont des entiers tels qu'ils donnent lieu au poids moléculaire tel que celui mentionné ci-dessus ;
(F) -(CF(CF₃)CF₂O)_{j"}-
j" étant un entier tel qu'il donne lieu au poids moléculaire ci-dessus.

3. Composés selon la revendication 2, dans lesquels les structures R_{f} sont (A) ou (B).

4. Utilisation des composés selon les revendications 1 à 3 en tant qu'agents stabilisants thermiques pour des huiles et des graisses fluorées dans des conditions thermo-oxydantes en présence de métaux.

5. Utilisation des composés selon les revendications 1 à 3 en tant qu'additifs anti-rouille pour des huiles et des graisses fluorées.

6. Utilisation selon la revendication 4 en tant qu'additifs anti-rouille.

7. Compositions lubrifiantes comprenant :
- de 99,95 à 90 % en poids, de préférence de 99,5 à 95 %, d'une huile de perfluoropolyéther ou d'une graisse à base de PFPE sur des huiles de perfluoropolyéther ;
- de 0,05 à 10 % en poids, de préférence de 0,5 à 5 % en poids, d'au moins l'un des composés triazine de formule (I) selon les revendications 1 à 3.

8. Compositions selon la revendication 7, dans lesquelles l'huile de perfluoropolyéther est choisie parmi les classes suivantes :
(1) E-O-[CF₂CF(CF₃)O]_{m'}(CFXO)_{n'}-E'
dans laquelle :
X est un groupe -F ou un groupe -CF₃ ;
E et E', identiques ou différents l'un de l'autre, sont choisis parmi un groupe -CF₃, un groupe -C₂F₅ ou un groupe -C₃F₇ ;
m' et n' sont des entiers tels que le rapport m'/n' est compris entre 20 et 1000, n' étant différent de 0, et la viscosité du produit à 20°C est comprise entre 10 et 4000 cSt ; les motifs étant distribués statistiquement le long du squelette ;
(2) C₃F₇O-[CF(CF₃)CF₂O]_{0'}-D
dans laquelle
D est un groupe -C₂F₅ ou un groupe -C₃F₇ ;
o' est un entier tel que la viscosité du produit soit dans la plage indiquée en (1) ;
(3) {C₃F₇O-[CF(CF₃)CF₂O]_{p'}-CF(CF₃)-}₂
dans laquelle
p' est un entier tel que la viscosité du produit soit dans la plage indiquée en (1) ;
(4) E-O-[CF₂CF(CF₃)O]_{q'}(C₂F₄O)_{r'}(CFX)_{s'}-E'
dans laquelle
X est un groupe -F ou un groupe -CF₃ ;
E et E', identiques ou différents l'un de l'autre, sont choisis parmi un groupe -CF₃, un groupe -C₂F₅ ou un groupe -C₃F₇ ;
q', r' et s' sont des entiers, y compris 0, de telle sorte que la viscosité du produit soit dans la plage indiquée en (1) ;
(5) E-O-(C₂F₄O)_{t'}(CF₂O)_{u'}-E'
dans laquelle
E et E', identiques ou différents l'un de l'autre, sont choisis parmi un groupe -CF₃, un groupe -C₂F₅ ou un groupe -C₃F₇ ;
t' et u' sont des entiers tels que le rapport t'/u' soit compris entre 0,1 et 5, u' étant différent de 0, et la viscosité du produit est dans la plage signalée ci-dessus en (1) ;
(6) E-O-(CF₂CF₂CF₂O)_{v'}-E'
dans laquelle :
E et E', identiques ou différents l'un de l'autre, sont choisis parmi un groupe -CF₃, un groupe -C₂F₅ ou un groupe -C₃F₇ ;
v' est un nombre tel que la viscosité du produit soit dans la plage signalée ci-dessus en (1).
(7) D-O-(CF₂CF₂O)_{z'}-D'
dans laquelle
D et D', identiques ou différents l'un de l'autre, sont choisis parmi un groupe -C₂F₅ ou un groupe -C₃F₇ ;
z' est un entier tel que la viscosité du produit soit dans la plage signalée ci-dessus en (1).
(8) E₁-O-(CF₂O)ₙ(CF₂CF₂O)ₘ-(CF₂CF₂CF₂O)ₚ(CF₂CF₂CF₂CF₂O)_{q}-E₂
dans laquelle
E₁ et E₂ sont des groupes terminaux perfluoroalkyle identiques ou différents l'un de l'autre, de formule -(CF₂)_{z}CF₃, dans laquelle z est un entier de 0 à 3 ; n, m, p, q sont des entiers tels que la viscosité soit telle que définie en (1), m/n est compris entre 2 et 20, n étant différent de 0, de préférence compris entre 2 et 10 ; le rapport (p+q)/(m+n+p+q) est compris entre 0,05 et 0,2, (m+n+p+q) étant différent de 0 ; n/(m+n+q+p) s'échelonne entre 0,05 et 0,4 (m+n+p+q) étant différent de 0.

9. Compositions selon la revendication 8, dans lesquelles les huiles de perfluoropolyéther sont celles des classes (1), (4), (5) et (8).

10. Compositions selon les revendications 7 à 9, comprenant les additifs couramment utilisés dans des formulations lubrifiantes de perfluoropolyéther, de préférence des additifs anti-usure.

11. Procédé de préparation de composés triazine de formule (I) selon les revendications 1 à 3, comprenant les stades suivants :
STADE A)
i) la réaction d'un dérivé de perfluoropolyoxyalkylène de formule
T"₁-CFW₁-O-R_{f}-CFW₂-T"₂ (II)
dans laquelle
R_{f}, W₁ et W₂ présentent la signification ci-dessus ;
T"₁ et T"₂ peuvent être identiques ou différents l'un de l'autre, de formule générale -CHAₐ-Bₐ(CH₂CH₂O)ₙₐ-H, dans laquelle Aₐ est un atome d'hydrogène, un groupe CF₃ ; Bₐ est un atome d'oxygène, un atome de soufre, un groupe NH ; na est un entier de 0 à 6, les extrêmes étant inclus ; ou choisis parmi un atome de fluor, un groupe CF₃, un groupe C₂F₅ ou un groupe (C₂F₄)Cl, à condition qu'au moins l'un des deux groupes terminaux T"₁ et T"₂ soit un groupe CHAₐ-Bₐ(CH₂CH₂O)ₙₐ-H, de préférence choisi parmi un groupe O-CH₂OH, un groupe O-CH₂SH, un groupe O-CH₂NH₂, un groupe CH(OH)CF₃ ;
avec
une trihalogéno-triazine de formule : dans laquelle J est un atome de chlore, un atome de fluor, de préférence un atome de chlore ;
à une température comprise entre 0° et 10°C, où le rapport entre les équivalents du composé (II) et les moles de (III) est égal à 1:1, en présence d'un solvant inerte dans les conditions de réaction, capable de solubiliser les réactifs, et en présence d'une base organique ou inorganique, en maintenant de préférence le mélange réactionnel sous agitation ;
ii) la réaction du produit obtenu en i) avec un équivalent d'un dérivé de formule :
Q-H (IV)
dans laquelle Q présente la signification signalée ci-dessus pour Q₁ et Q₂ ;
à une température dans la plage de 25° à 35°C ;
iii) la réaction du produit obtenu en ii) avec un équivalent d'un composé de formule (IV), identique ou différent de celui utilisé dans l'étape ii), à une température dans la plage de 65°C à 100°C, de préférence de 70°C à 90°C ;
STADE B)
la séparation de la phase organique du mélange réactionnel obtenu en A) de la phase aqueuse et la séparation subséquente, de préférence par filtration, de la phase organique en vue d'éliminer les sels insolubles organiques ou inorganiques résiduels ;
STADE C)
plusieurs lavages de la phase organique liquide avec de l'eau acide et la séparation subséquente du composé obtenu de formule (I) du solvant organique, par exemple, par évaporation.

12. Procédé selon la revendication 11, dans lequel dans le stade A), le solvant inerte est choisi parmi le toluène, le xylène, l'hexafluoroxylène, l'acétone, la diéthylcétone.

13. Procédé selon les revendications 11 à 12, dans lequel dans le stade A), la base inorganique est choisie parmi le NaOH, le KOH, le Na₂CO₃, le K₂CO₃ ; la base organique est choisie parmi la 2,6-diméthylpyridine, la 2-méthylquinoléine, la 2,4,6-triméthylpyridine (collidine).

14. Procédé selon les revendications 11 à 13, dans lequel la base est la 2,4,6-triméthylpyridine.

15. Procédé selon les revendications 11 à 14, dans lequel le rapport entre les équivalents de base et la somme des équivalents des composés (II) et (IV) utilisés dans les trois étapes du stade (A) est dans la plage de 1:1 à 2:1, de préférence de 1:1 à 1,5:1.

16. Graisses lubrifiantes présentant une base de perfluoropolyéther comprenant l'additif selon les revendications 1 à 3, une huile de perfluoropolyéther et un agent épaississant, de préférence choisi parmi le PTFE, le téréphtalamate de sodium, des savons de calcium ou de lithium, la polyurée, plus préférablement le PTFE.

17. Graisses selon la revendication 16, comprenant du talc, des charges inorganiques, des additifs anti-usure.
